

## UNITED STATES PATENT OFFICE

KARL B. THEWS, OF DREXEL HILL, AND JOSEPH S. CARLITZ, OF PHILADELPHIA, PENNSYLVANIA; SAID CARLITZ ASSIGNOR TO SAID THEWS

## TREATMENT OF IRON OR STEEL

No Drawing.

Application filed December 7, 1929. Serial No. 412,565.

This invention relates to a process for reducing the dissolution of iron and steel during the removal of iron oxide or scale in pickling baths of sulphuric or other acids. 5 The methods disclosed herein are also useful in preventing corrosion of iron and steel containers of such acids.

Heretofore it has been customary to use various inhibiting agents in the pickling 10 baths to prevent pitting or etching of the surface of the iron or steel. These substances have been more or less successful in the attainment of such results, the best of these inhibitors so far used apparently being the 15 substitution products of normal thiourea of which the ditolyl derivatives are the most effective.

It is the object of this invention to improve the processes heretofore used by the use as 20 inhibitors of derivatives of selenium and tellurium which are found to be generally superior to the corresponding sulphur derivatives.

The attainment of the object outlined above 25 and the more specific objects of the invention will be clear from the following description.

It is found that a greatly improved inhibiting action results if instead of the derivatives of normal thiourea, there are used derivatives of normal selenourea or tellurourea. 30 The derivatives include compounds having the general formula:

35



in which X represents either selenium or tellurium and R represents hydrogen, or an alkyl, aryl or acyl group, or in which two R's 40 may be replaced by an ethylene, or the like, derivative connected by two bonds to the same or different nitrogen atoms.

As examples of suitable alkyl groups, there 45 may be cited methyl, ethyl, propyl, butyl,

amyl, etc., propyl, butyl, amyl and higher radicals being of any of the various isomeric types, such as normal, iso-, tertiary, etc. Substituted alkyl groups may also be used, in which, for example, one or more hydrogen 50 atoms are replaced by amino, sulphonic, nitro, or other groups.

The aryl groups may be joined to the nitrogen atoms either at the nucleus or side chain. Of the first type, phenyl, tolyl, xylyl,  $\alpha$  or  $\beta$  55 naphthyl, etc. are examples. The junction to the nitrogen atoms may take place at any of the unsubstituted carbon atoms. Of the second type, benzyl is the best example. Here again there may be various groups replacing 60 the hydrogen atoms in either the nucleus or side chains.

The acyl groups may be formyl, acetyl, propionyl, benzoyl, phthalyl, succinyl, etc., or 65 substituted derivatives thereof.

While only one monosubstitution derivative of either normal selenourea or normal tellurourea may be formed, it will be obvious from the structural formula given above that either 1, 2 or 1, 3 distribution products may 70 be formed depending upon whether the substituent groups are in the same or different amino groups. The two substituents may be either the same or different; if different both may be of alkyl, aryl or acyl types or they 75 may be of different types: for example, 1-methyl 3-p-tolyl selenourea, and 1, 2 dibenzyl tellurourea are disubstitution products illustrative of these types.

As to trisubstitution products, it is necessary 80 that two of the substituent groups be attached to one nitrogen atom and one to the other. Of these groups all may be the same, two the same, or all different and of the same or different types. Similarly, where there are four substituent groups, there may be duplication or all may be different.

There may also be used derivatives in which 85 the two nitrogen atoms are joined to a single radical, each by a single linkage, or in which 90

one of the nitrogen atoms is joined to a radical by a double linkage. The radicals in these cases may be either alkyl, aryl, or acyl. As an example there may be cited the phthalyl derivative:



10 It will be seen that this compound may be considered to be a derivative of phthalimide. An analogous derivative of succinimide is an example of an aliphatic acyl derivative. An ethylene, propylene or similar radical may 15 enter a similar position to form an alkylene derivative. The different nitrogen groups may be joined to the bonds of a bivalent radical such as phthalyl, succinyl, ethylene, or propylene. It will be understood that where 20 the term "alkyl" is used, it is in a broad sense so as to include not only alkylene groups, such as ethylene, but also heterocyclic derivatives such as terpene groups. The terms "aryl" and "acyl" are intended to have similar broad 25 interpretations, the term "aryl", for example, being intended to include "aralkyl" such as benzyl.

In a general way, it may be said that the operative substances are represented by the 30 general formula above in which one or more of the R's represents an organic radical or hydrogen, and in which X represents Se or Te. It appears that the inhibiting action to a greater or less degree is characteristic of 35 this class of compounds.

The mechanism of the process involved in using these substances is similar to that usually used. The pickling solution may contain sulphuric or other suitable acidic materials such as are now used in effective concentrations. For example, approximately 40 10% sulphuric acid solution in water may be used. To such pickling solution up to approximately 1% of one of the inhibiting 45 agents is added. The pickling is then effected in the usual fashion by submerging the iron or steel articles in the solution either at ordinary or elevated temperatures. In cases where it is desired to protect a tank 50 against acid which is contained therein, the inhibiting agent is added to the acid.

While the derivatives are by far the most effective, normal selenourea and normal tellurourea both exert an appreciable inhibiting action and they are therefore considered 55 to be within the scope of the invention. Of the various derivatives, the alkyl and aryl are generally found to be best; the acyl derivatives are less effective but more so than 60 the corresponding thiourea derivatives.

For convenience in handling the inhibiting substances in the small quantities necessary in a pickling bath, it may be desirable to mix them with a large proportion of a 65 carrier substance which may be of such na-

ture as to assist the pickling action, for example, sodium chloride or sodium bisulphate. Mixtures of various inhibiting agents may also be used.

The various derivatives referred to are best 70 prepared by the general methods well known to the art. In general it may be stated that the seleno- and tellurourea derivatives are prepared similarly to the corresponding thiourea derivatives although special methods of preparation are well known to the art. In view of the fact that the preparations of the derivatives form no part of the instant invention, they have not been discussed in detail. 75

What we claim and desire to protect by Letters Patent is:

1. An aqueous solution of a non-oxidizing acid capable of dissolving iron oxides to which has been added an inhibitor comprising an organic substitution product of CX(NH<sub>2</sub>)<sub>2</sub>, in which X represents Se or Te. 85

2. An aqueous solution of a non-oxidizing acid capable of dissolving iron oxides to which has been added an inhibitor comprising an organic substitution product or selenourea. 90

3. An aqueous solution of a non-oxidizing acid capable of dissolving iron oxides to which has been added an inhibitor comprising a substance having the general formula CX(NR<sub>2</sub>)<sub>2</sub>, in which X represents Se or Te, and R represents hydrogen or an alkyl, aryl or acyl group. 95

4. An aqueous solution of a non-oxidizing acid capable of dissolving iron oxides to which has been added an inhibitor comprising a substance having the general formula CSe(NR<sub>2</sub>)<sub>2</sub>, in which R represents hydrogen, or an alkyl, aryl or acyl group. 100

5. The process of pickling iron and steel products which consists in treating said products with an aqueous solution of a non-oxidizing acid capable of dissolving iron oxides to which has been added an inhibitor comprising an organic substitution product of CX(NH<sub>2</sub>)<sub>2</sub>, in which X represents Se or Te. 110

6. The process of pickling iron and steel products which consists in treating said products with an aqueous solution of a non-oxidizing acid capable of dissolving iron oxides to which has been added an inhibitor comprising an organic substitution product of selenourea. 115

7. The process of pickling iron and steel products which consists in treating said products with an aqueous solution of a non-oxidizing acid capable of dissolving iron oxides to which has been added an inhibitor comprising a substance having the general formula CX(NR<sub>2</sub>)<sub>2</sub>, in which X represents Se or Te, and R represents hydrogen or an alkyl, aryl or acyl group. 120

8. The process of pickling iron and steel products which consists in treating said prod- 125

ucts with an aqueous solution of a non-oxidizing acid capable of dissolving iron oxides to which has been added an inhibitor comprising a substance having the general formula CSe(NR<sub>2</sub>)<sub>2</sub>, in which R represents hydrogen, 5 or an alkyl, aryl or acyl group.

In testimony of which invention, we have hereunto set our hands, at Philadelphia, Pennsylvania, on this 6th day of December, 1929.

10 KARL B. THEWS.  
JOSEPH S. CARLITZ.

15

3

## CERTIFICATE OF CORRECTION.

20 Patent No. 1,759,634.

Granted May 20, 1930, to

KARL B. THEWS ET AL.

25 It is hereby certified that error appears in the printed specification of the above numbered patent requiring correction as follows: Page 2, line 88, claim 2, for the word "an" second occurrence read "a", and line 91, for "or" read "of"; 30 and that the said Letters Patent should be read with these corrections therein that the same may conform to the record of the case in the Patent Office.

Signed and sealed this 24th day of June, A. D. 1930.

35

M. J. Moore,  
Acting Commissioner of Patents.

(Seal) 148-8

40

45

50

55

60

65